

1

2,972,590

**COMPOSITION OF MATTER AND PROCESS FOR OBTAINING SAME**

Joseph Cunder, East Orange, and Francis J. Licata, West Caldwell, N.J., assignors to Nopco Chemical Company, Harrison, N.J., a corporation of New Jersey

No Drawing. Filed Feb. 21, 1958, Ser. No. 716,547

6 Claims. (Cl. 260—18)

The present invention relates to novel metallic soap products. More particularly, the present invention relates to metallic soap products that have great utility in compositions such as sanding sealers, lacquers and the like.

Use of metal soaps in sanding sealers, lacquers and varnish compositions is well known and has been practiced by the art for many years. Sanding sealers are lacquer type coatings which are primarily employed to seal porous surfaces such as wood and are designed to prevent raising of wood grain. Zinc stearate is usually added to sanding sealer compositions in order to permit clean and easy sanding by acting as a lubricant and by retarding the gumming of the sandpaper during the sanding step. Lacquer and varnish compositions when applied to surfaces result in a glossy finish. In many instances, a dull or matte finish is preferred. Such dull finishes are provided for by incorporating into the lacquer or varnish composition finely divided microscopic particles. Materials which are added for the purpose of bringing about dull or matte finishes are known as flattening agents. Well-known flattening agents are, for instance, metallic soaps such as zinc stearate, zinc palmitate, calcium stearate and magnesium stearate.

However, in order to use these various metallic soaps as additives to sanding sealers, lacquers and varnishes, it is necessary to first grind them in order to disintegrate or break down the clusters of the soap into their individual particles. Generally, the soaps are ground in the presence of a hydrocarbon solvent or in the presence of a portion of the vehicle to which they are to be added. Pebble mills may be employed for grinding and their use involves grinding periods for up to twenty hours. Such grinding procedures involve unavoidably long periods of time as well as involving the extra manipulative step plus the necessary grinding equipment. Also, in many instances, heat generated during grinding procedures may cause discoloration of the various soaps. It has also been found in the case of zinc soaps, particularly due to their extreme fineness and large surface area, that they contain a large volume of air which in many instances during grinding becomes emulsified. This produces very rigid foams which cannot be poured out of the pebble mills.

Additionally, metallic soaps as presently employed bring about undesirable thickening of the vehicle when too high a concentration of soap is employed. Hence, the solids concentration is usually kept low to avoid this thickening, but, in many instances this results in films having poor weathering qualities because of the small amount of metallic soap present. These metallic soaps are, of course, known for their water-proofing properties.

Accordingly, it is an object of the present invention to obtain improved compositions of metallic soaps.

It is a further object to obtain improved metallic soaps in finely divided form which are useful in sanding sealers, lacquers, varnishes and the like.

2

It is another object to obtain improved metallic soaps in finely divided form that are useful as flattening agents.

It is a still further object to prepare finely divided metallic soaps useful as additives to the aforementioned vehicles without the necessity of grinding the soaps in order to obtain them in finely divided particles.

A further object is to obtain improved compositions of metallic soaps that may be used in increased quantities in organic vehicles such as varnishes and lacquers, without detracting from the stability, color or freely flowing properties of such vehicles and which may be added to such vehicles by simple mixing.

Further objects will become apparent from the detailed description given hereinafter. It is intended, however, that the detailed description and the specific examples do not limit the invention, but merely indicate the preferred embodiments of the invention since various changes and modifications within the scope of the invention will become apparent to those skilled in the art.

20 The above and other objects are accomplished in the following manner. It has unexpectedly been discovered that when a water-soluble soap is precipitated with a water-soluble zinc salt in the presence of an epoxy resin or ester thereof, to be described hereinafter, or when a

25 zinc soap is admixed with said epoxy resin or ester thereof, a product is obtained which is a uniform mixture of a zinc soap and resin or ester thereof and has the following unexpected characteristics. The product is in a finely divided state and after grinding to form optimum particle size may be added directly to a vehicle without further mechanical grinding. It may be added in increased quantities to such vehicles without in any manner decreasing or affecting the fluidity of freely flowing properties of the mixture which may be a sanding sealer, lacquer

30 or varnish composition. These compositions are of good color and stable and moreover, because increased quantities of metallic soap may be incorporated therein, they have improved waterproofing characteristics as well.

35 The resins may be described as resinous epoxides which are polyether derivatives of a dihydroxy aryl compound having alternating aliphatic chains and aromatic nuclei united through ether oxygen and being free from functional groups other than epoxy and hydroxyl groups. They may be prepared by reacting a dihydroxy aryl com-

40 pound, e.g., a dihydroxydiphenyl alkane, with a halohydrin in the presence of alkali at elevated temperatures. Suitable aryl materials are p,p'-dihydroxydiphenyl dimethyl methane; p,p'-dihydroxydiphenyl; resorcinol; bis(4-hydroxyphenyl)-1,1 ethane; bis(4-hydroxyphenyl)-

45 1,1-isobutane; bis(4-hydroxyphenyl)-2,2-butane; bis(4-hydroxy-2-methylphenyl)-2,2-propane; bis(2-hydroxy-naphthyl)-methane while suitable halohydrins are epichlorohydrin, and dichlorohydrins such as 1,3 dichloro-2-hydroxy propane and 1,2-dichloro-3-hydroxy propane.

50 55 These resins are prepared by heating the halohydrin and dihydric phenol for several hours at elevated temperatures of e.g., 50° to 150° C. When epichlorohydrin and a dihydric phenol are reacted, they may be present in a ratio of from about one to two mols of epichlorohydrin

60 per mol of dihydric phenol. A base such as sodium or potassium hydroxide is also present in an amount sufficient to neutralize the acid formed during reaction. Generally an excess of base is present e.g., 1.1 to 1.3 chemical equivalents of base per mol of epichlorohydrin.

65 65 When epichlorohydrin and bis(4-hydroxyphenyl) dimethyl methane, also referred to as bisphenol-A, are reacted together, materials generally believed to have the structure



are obtained where  $n$  represents the extent of polymerization. When the mol ratio of epichlorohydrin to phenol is 2:1,  $n$  is zero and the molecular weight is 340 according to theory, although in practice some polymerization occurs thereby accounting for an  $n$  value somewhat higher than zero and a molecular weight somewhat above theoretical calculations. The value of  $n$  may extend up to for instance 13 corresponding to a molecular weight of about 4,000.

A number of these resins are available commercially and are listed below, the data being obtained from "Epoxy Resins" by Lee and Neville, McGraw-Hill Publishing Co., Inc. 1957 (page 20).

| Epon Resin (Shell Chemical Co.) No. | M.E., °C.<br>(Durrans Method) | Epoxide Equivalent | Av. Molecular Wt. |
|-------------------------------------|-------------------------------|--------------------|-------------------|
| 828                                 | Liquid (at R.T.)              | 175-210            | 350-400           |
| 834                                 | Liquid (at R.T.)              | 225-290            | 450               |
| 864                                 | 40-50                         | 300-375            | 700               |
| 1001                                | 64-76                         | 450-525            | 900-1,000         |
| 1004                                | 95-105                        | 870-1,025          | 1,400             |
| 1007                                | 125-132                       | 1,650-2,050        | 2,900             |

It is of course understood that the above epoxy resins are not the only epoxy resins that may be employed herein. They are merely exemplary of the various commercially available materials useful within the scope of this invention since other epoxy resins are obtainable when, in lieu of the aforementioned polyhydroxy aryl compounds, other polyhydroxy materials such as ethylene glycol, diethylene glycol, glycerine, etc. are used.

It is to be understood that the preparation of the epoxy resins and esters thereof are not part of this invention and the invention is not limited to resins obtained by any one particular method. Additionally, other resins such as epoxy resin esters have been found to be suitable in the present invention. They are prepared by reacting the epoxy resin with a fatty acid to bring about esterification of the resin. Suitable fatty acids are saturated and unsaturated monocarboxylic fatty acids having from 8 to 22 carbon atoms such as caprylic, ethyl hexoic, palmitic, stearic, arachidic, behenic, oleic, linoleic acids etc., and mixtures thereof as well as naturally occurring sources thereof, e.g., soybean fatty acids, linseed fatty acids, castor fatty acids, coconut fatty acids, etc.

To prepare the novel flattening agents, a fatty acid is first saponified alone, or in the presence of the resin which is uniformly dispersed throughout the solution. Any suitable saturated fatty acid may be used as the starting material i.e., saturated aliphatic monocarboxylic acids having from about 8 to 22 carbon atoms such as palmitic, stearic, arachidic, behenic, caprylic or ethyl hexoic acids and their mixtures, fatty acids obtained by splitting glycerides and mixtures thereof such as tallow, hydrogenated fish oils, e.g., hydrogenated sardine oil, hydrogenated vegetable oils e.g., hydrogenated soy bean oil, hydrogenated castor oil, hydrogenated cottonseed oil and hydrogenated coconut oil.

Processes for the conversion of fatty acids or glycerides if such are used, into water-soluble soaps using an alkali are well known in the art. Generally, saponification is accomplished by reacting the fatty acid or glyceride with a base such as sodium, potassium or ammonium hydroxide in the presence of water. Since water-soluble soaps produced by any of the prior art processes are fully suited for use in the present invention, nothing herein should be construed as limiting the present invention to the use of soaps obtained by any one particular method.

Thereafter, a water-soluble zinc salt is added to the resulting water-soluble soap solution which also contains the epoxy resin. If the resin was not present during saponification, it may be added prior to or with the addition of the water-soluble zinc salt. This addition brings about precipitation of the soap as a zinc soap containing the resin uniformly dispersed throughout the soap. Al-

ternatively, the zinc salt may be added to a solution or dispersion of the water-soluble soap in the absence of the resin which may be subsequently admixed with the resulting zinc soap.

- 5 The quantity of zinc salt employed to accomplish precipitation should be at least sufficient to react with all of the water-soluble soap present. While the use of a stoichiometrically equivalent quantity of zinc salt solution should obviate the possibility that any water-soluble 10 soap will be occluded in the precipitated product, an excess quantity can be and is at times preferably employed. Suitable salts are zinc sulfate, zinc chloride, zinc acetate, etc.

Precipitation is accomplished by adding a heated aqueous 15 solution of the water-soluble zinc salt to the solution or dispersion of the soap with or without the presence of the resin. If desired, this sequence can be reversed. The zinc salts previously recited are not limiting since other zinc salts may be used provided they are 20 soluble in water at the temperature which they are to be used and provided further that these salts will form water-insoluble compounds with the water-soluble soaps. Generally the solution of the metal salt precipitant contains from 5% to 40% by weight of zinc salt. Preferably about 20% zinc salt solutions are used. However, if any, upon the precipitated composition. The salt solution when added is usually at an elevated temperature e.g., from about 50° C. to about 95° C. and the soap 30 solution may likewise be at the same elevated temperature.

After the desired composition has been precipitated, it can be separated from the aqueous solution in which it is dispersed by any convenient means. Usually, this step 35 is accomplished by passing the dispersion through a filter. The filtered product is subsequently washed several times in water to remove residual water-soluble salts present. The washing step is ordinarily carried out in water heated to a temperature of from about 40° C. to about 70° C. 40 After washing, the product is dried, generally in an oven heated to a temperature of from about 100° F. to 180° F., and subsequently ground by appropriate means to obtain optimum particle size. If the zinc soap was obtained in the absence of the resin, such may now be 45 added by any convenient mixing means, e.g., hammer type mill. The resulting product which, as stated before, is a uniform mixture of a zinc soap and resin or ester thereof, although insoluble and not dispersible in water, is highly dispersible in organic solvents and other organic 50 vehicles used in e.g., sanding sealer, lacquer or varnish compositions. As aforesaid, the addition of the novel products of the present invention to these solvents or vehicles is accomplished by simple mixing without resorting to grinding and these products may be present 55 in amounts not heretofore possible to employ.

The quantity of epoxy resin or ester thereof may vary and may be from about 1/2% to 20% by weight based upon the weight of the fatty acid used. Preferably 5% by weight based upon the weight of the fatty acid is used.

60 Additionally, the solid composition may contain in minor amounts other constituents such as plasticizers, softeners, pigments, dyes and the like. Generally, when the novel products described herein are employed as flattening agents, they may be present in 65 a lacquer in an amount of from 1/2% to 10% by weight of the lacquer. If they are to be employed in sanding sealers, they may be also present in an amount of from 1/2% to 10% by weight of the vehicle. If desired, however, up to 25% of these novel soaps may be satisfactorily 70 employed in the various vehicles.

For a fuller understanding of the nature and objects of the present invention, reference may be made to the following examples which are given merely to illustrate the invention and are not to be construed in a limiting sense, all parts given being by weight.

*Example I*

950 parts of stearic acid and 50 parts of Shell Epon Resin 864 were melted together in the presence of 2000 parts of water at a temperature of 80° C. to 95° C. Thereafter 157 parts of dry sodium hydroxide dissolved in water to form a 50% by weight solution were added to the molten aqueous mixture of stearic acid and resin in order to saponify the acid. The resulting soap, resin mixture was diluted with water to form a 6% by weight concentration thereof based on the weight of the soap. To this solution, 375 parts of zinc sulfate monohydrate dissolved in water to form a 20% by weight solution of zinc sulfate monohydrate were slowly added during one hour to bring about precipitation of the sodium stearate soap as zinc stearate containing the resin uniformly dispersed throughout the zinc stearate. This was accomplished at a temperature of 80° to 85° C. The resulting precipitate which comprised a mixture of zinc stearate and resin was filtered off from the mother liquor and washed free of sulfates. The precipitate was dried at 140° F. and ground through a  $\frac{1}{64}$  inch screen.

The following data were determined upon analysis of the composition of Example I, all percents being by weight.

## Percent:

|             |      |
|-------------|------|
| Moisture    | 0.5  |
| Washed ash  | 14.4 |
| Soluble ash | 0.3  |

*Example II*

To illustrate the use of our novel metal soaps as flattening agents, 1.4 parts of the product of Example I were stirred into 98.6 parts of a lacquer referred to as C.M.L. XE1510 lacquer, a product of the Coating Materials Laboratory, Belleville, New Jersey. No grinding of the soap into the vehicle was carried out. The resulting product was a homogeneous dispersion. A portion was applied to a glass plate and the resulting film was found to be smooth with a minimum of agglomerations, i.e., it compared favorably with films prepared from lacquers having the flattening agent ground in e.g., with a pebble mill.

The C.M.L. lacquer was prepared as follows. First, two mixes were prepared. Mix A contained 100 parts by weight of one-half second nitrocellulose and 60 parts by weight of modified maleic resin (Arochem 520 having an acid number of 25-35 and a melting point of 140-145° C.). Mix B contained 15 parts by weight ethanol, 50 parts by weight toluene and 35 parts by weight butyl acetate. Then the final composition was made by mixing together 20 parts by weight of Mix A with 80 parts by weight of Mix B.

Of course, lacquers containing other film formers besides nitrocellulose may be used such as cellulose acetate and synthetic resins such as urea-formaldehyde resin or alkyd resins.

*Example III*

95 parts of double pressed stearic acid and 5 parts of Shell Epon Resin 1001 were melted together in the presence of 200 parts of water at a temperature of 80° to 95° C. 15.7 parts of dry sodium hydroxide, dissolved in 15.7 parts of water were added to the molten stearic acid, resin mixture in order to saponify the acid. The resulting soap, resin mixture was diluted to 2000 parts of water to form about 5% concentration thereof based on the weight of the soap. To this solution 37.5 parts of zinc sulfate monohydrate dissolved in water to form a 20% by weight solution of zinc sulfate monohydrate were slowly added during one hour to precipitate the sodium stearate soap as zinc stearate containing the resin uniformly dispersed throughout the zinc stearate. This was accomplished at a temperature of 80° to 85° C. The resulting precipitate which comprised a mixture of zinc stearate and resin was filtered off from the mother liquor and washed free of sulfates. The precipitate was

stearate and resin was filtered off from the mother liquor and washed free of sulfates. The precipitate was dried at 140° F. and ground through a  $\frac{1}{64}$  inch screen.

*Example IV*

95 parts of double pressed stearic acid and 5 parts of Shell Epon Resin 828 were melted together in the presence of 200 parts of water at a temperature of 80° to 95° C. 15.7 parts of dry sodium hydroxide, dissolved in 15.7 parts of water were added to the molten stearic acid, resin mixture in order to saponify the acid. The resulting soap, resin mixture was diluted to 2000 parts of water to form about 5% concentration thereof based on the weight of the soap. To this solution 37.5 parts of zinc sulfate monohydrate dissolved in water to form a 20% by weight solution of zinc sulfate monohydrate were slowly added during one hour to precipitate the sodium stearate soap as zinc stearate containing the resin uniformly dispersed throughout the zinc stearate. This was accomplished at a temperature of 80° to 85° C. The resulting precipitate which comprised a mixture of zinc stearate and resin was filtered off from the mother liquor and washed free of sulfates. The precipitate was dried at 140° F. and ground through a  $\frac{1}{64}$  inch screen.

*Example V*

95 parts of double pressed stearic acid and 5 parts of Shell Epon Resin 1004 were melted together in the presence of 200 parts of water at a temperature of 80° to 95° C. 15.7 parts of dry sodium hydroxide, dissolved in 15.7 parts of water were added to the molten stearic acid, resin mixture in order to saponify the acid. The resulting soap, resin mixture was diluted to 2000 parts of water to form about 5% concentration thereof based on the weight of the soap. To this solution 37.5 parts of zinc sulfate monohydrate dissolved in water to form a 20% by weight solution of zinc sulfate monohydrate were slowly added during one hour to precipitate the sodium stearate soap as zinc stearate containing the resin uniformly dispersed throughout the zinc stearate. This was accomplished at a temperature of 80° to 85° C. The resulting precipitate which comprised a mixture of zinc stearate and resin was filtered off from the mother liquor and washed free of sulfates. The precipitate was dried at 140° F. and ground through a  $\frac{1}{64}$  inch screen.

*Example VI*

99 parts of double pressed stearic acid and 1 part of Shell Epon Resin 1001 were melted together in the presence of 200 parts of water at a temperature of 80° to 95° C. 15.7 parts of dry sodium hydroxide, dissolved in 15.7 parts of water were added to the molten stearic acid, resin mixture in order to saponify the acid. The resulting soap, resin mixture was diluted to 2000 parts of water to form about 5% concentration thereof based on the weight of the soap. To this solution 37.5 parts of zinc sulfate monohydrate dissolved in water to form a 20% by weight solution of zinc sulfate monohydrate were slowly added during one hour to precipitate the sodium stearate soap as zinc stearate containing the resin uniformly dispersed throughout the zinc stearate. This was accomplished at a temperature of 80° to 85° C. The resulting precipitate which comprised a mixture of zinc stearate and resin was filtered off from the mother liquor and washed free of sulfates. The precipitate was dried at 140° F. and ground through a  $\frac{1}{64}$  inch screen.

*Example VII*

97 parts of double pressed stearic acid and 3 parts of Shell Epon Resin 1001 were melted together in the presence of 200 parts of water at a temperature of 80° to 95° C. 15.7 parts of dry sodium hydroxide, dissolved in 15.7 parts of water were added to the molten stearic acid, resin mixture in order to saponify the acid. The resulting soap, resin mixture was diluted to 2000 parts of water to form about 5% concentration thereof based

on the weight of the soap. To this solution 37.5 parts of zinc sulfate monohydrate dissolved in water to form a 20% by weight solution of the zinc sulfate monohydrate were slowly added during one hour to precipitate the sodium stearate soap as zinc stearate containing the resin uniformly dispersed throughout the zinc stearate. This was accomplished at a temperature of 80° to 85° C. The resulting precipitate which comprised a mixture of zinc stearate and resin was filtered off from the mother liquor and washed free of sulfates. The precipitate was dried at 140° F. and ground through a  $\frac{1}{64}$  inch screen.

*Example VIII*

990 parts of double pressed stearic acid and 10 parts of Shell Epon Resin 828 were melted together in the presence of 2000 parts of water at a temperature of 80° to 95° C. 157 parts of dry sodium hydroxide, dissolved in 157 parts of water were added to the molten stearic acid, resin mixture in order to saponify the acid. The resulting soap, resin mixture was diluted to 20,000 parts of water to form about 5% concentration thereof based on the weight of the soap. To this solution 375 parts of zinc sulfate monohydrate dissolved in water to form a 20% by weight solution of zinc sulfate monohydrate were slowly added during one hour to precipitate the sodium stearate soap as zinc stearate containing the resin uniformly dispersed throughout the zinc stearate. This was accomplished at a temperature of 80° to 85° C. The resulting precipitate which comprised a mixture of zinc stearate and resin was filtered off from the mother liquor and washed free of sulfates. The precipitate was dried at 140° F. and ground through a  $\frac{1}{64}$  inch screen.

*Example IX*

90 parts of double pressed stearic acid along with 10 parts of Shell Epon Resin 1001 were melted together in the presence of 200 parts of water at a temperature of 80° to 95° C. 15.7 parts of dry sodium hydroxide, dissolved in 15.7 parts of water were added to the molten stearic acid, resin mixture in order to saponify the acid. The resulting soap, resin mixture was diluted to 2000 parts of water to form about 5% concentration thereof based on the weight of the soap. To this solution 37.5 parts of zinc sulfate monohydrate were slowly added during one hour to precipitate the sodium stearate soap as zinc stearate containing the resin uniformly dispersed throughout the zinc stearate. This was accomplished at a temperature of 80° to 85° C. The resulting precipitate which comprised a mixture of zinc stearate and resin was filtered off from the mother liquor and washed free of sulfates. The precipitate was dried at 140° F. and ground through a  $\frac{1}{64}$  inch screen.

*Example X*

To 95 parts of melted stearic acid were added 15.7 parts of sodium hydroxide in the form of a 50% by weight aqueous solution in order to saponify the fatty acid. The resulting soap was diluted with water to form a 10% by weight concentration thereof. A 20% by weight aqueous solution of zinc sulfate monohydrate was prepared from

37.5 parts of zinc sulfate monohydrate. One third of this zinc sulfate solution was added to the soap solution to bring about partial precipitation. The temperature of the soap solution was maintained at about 210° F. Thereafter, 5 parts of an ester of Shell Epon Resin 1001 and stearic acid having an acid value of 20 was heated to about 210° and then slowly poured into the partially precipitated soap to effect a uniform dispersion of the resin. Finally the remainder of the zinc sulfate solution was added to complete precipitation at the same temperature. The precipitated material which comprised a mixture of zinc stearate and resin was filtered off from the mother liquor and washed free of sulfates. It was then dried at 150° F. and ground through a  $\frac{1}{64}$  inch screen.

Having described our invention what we claim as new and desire to secure by Letters Patent is:

1. A composition of matter comprising in admixture (1) zinc stearate and (2) a resin selected from the group consisting of an epoxy resin and esters thereof, said resin being present in an amount of from about  $\frac{1}{2}\%$  to 20% by weight based upon the weight of stearic acid from which said zinc stearate is derived.

2. A composition of matter comprising in admixture (1) zinc stearate and (2) a resin selected from the group consisting of a resinous epoxide which is a polyether derivative of a dihydroxy aryl compound having alternating aliphatic chains and aromatic nuclei united through ether oxygen and being free from functional groups other than epoxy and hydroxy groups and esters thereof, said resin being present in an amount of from about  $\frac{1}{2}\%$  to 20% by weight based upon the weight of stearic acid from which said zinc stearate is derived.

3. A composition of matter comprising in admixture, (1) zinc stearate and (2) an epoxy resin which is a condensation polymer of epichlorohydrin and p,p'-dihydroxy diphenyl dimethylmethane having a melting point of about 40° to 50° C., an epoxide equivalent of about 300 to 375 and an average molecular weight of about 700, said resin being present in an amount of about  $\frac{1}{2}\%$  to 20% by weight based upon the weight of stearic acid from which said zinc stearate is derived.

4. A composition of claim 3 in which said resin is present in an amount of about 5% by weight based upon the weight of stearic acid from which said zinc stearate is derived.

5. A freely flowing liquid composition comprising a lacquer and in an amount of from about  $\frac{1}{2}\%$  to 25% by weight thereof, the composition of claim 1.

6. A freely flowing liquid composition comprising a lacquer and in an amount of from about  $\frac{1}{2}\%$  to 25% by weight thereof, the composition of claim 3.

References Cited in the file of this patent

UNITED STATES PATENTS

2,803,609 Schlenker \_\_\_\_\_ Aug. 20, 1957

OTHER REFERENCES

Payne: "Organic Coating Technology," vol. I, pages 429-30, John Wiley & Sons, Inc., N.Y., 1954.